

## UNITED STATES PATENT OFFICE

1,934,730

## INTIMATE MIXTURE OR ALLOY

William S. Murray, Utica, and Daniel Gray,  
Oneida, N. Y., assignors to Oneida Community,  
Limited, Oneida, N. Y., a corporation of New  
York

No Drawing. Application July 22, 1930, Serial  
No. 469,913. Renewed January 31, 1933

3 Claims. (Cl. 75—1)

This invention relates to non-tarnishing metallic mixtures and alloys.

It is an object of the invention to produce an intimate metallic mixture or alloy which is tarnish-resisting and has a pleasant color.

An appreciable amount of indium added to silver produces an intimate mixture or alloy which has tarnish-resisting properties due to the indium. The indium, however, imparts a bluish tint or color to the silver and such color is considered objectionable particularly where the alloy is employed as a finish plating.

We have discovered that the addition of a third metal to the alloy produces an improvement in color and an intimate mixture of the elements. When the alloy or intimate mixture is used as a plating, it can be produced advantageously by plating the elements in superposed layers in alternate fashion and diffusing. While the elements may be plated individually or singly, in the present most advantageous practise, two of the elements are plated simultaneously from a plating bath, then the third metal is plated and finally by diffusing the plated layers there is produced an alloy or intimate mixture of the metals.

While various metals may be associated in the intimate mixture or alloy of the present invention, one advantageous combination is silver, gold and indium. In this alloy, the gold color counteracts the indium color and the alloy color simulates that of silver. This alloy may be produced by plating and, in the present preferred practise, the silver and gold are simultaneously plated from the same bath, the indium then plated thereon and the metals caused to mix intimately or alloy by diffusing.

In the simultaneous gold-silver plating, the anode of the bath is an alloy of gold and silver and the cathode is the base metal, such as nickel silver or even solid silver, to be plated simultaneously by the gold and silver. While the proportions of the metals in the anode may vary, as an example, the anode may contain 12½% gold and 87½% silver. The bath is advantageously a cyanide bath containing 8 ounces or more of free potassium cyanide salt per gallon, 0.6 to 1.0 ounces of gold in the form of a cyanide salt per gallon, and approximately 3.0 ounces of silver in the form of cyanide salt. The current density during the plating process is about 1/14 ampere per square inch. Under normal room temperatures, the process produces a good commercial plate containing about 12½% gold and 87½% silver.

The plating of indium on the gold-silver plate

is advantageously performed in a bath containing approximately 5 ounces (per gallon) of indium in the form of cyanide salts, about 9 ounces (per gallon) of free potassium cyanide and about 2½ ounces of sugars (dextrose). Insoluble anodes, such as carbon, are used in the process. With a current density of about 1/7 ampere per square inch, under normal temperatures, a good commercial deposit of indium is obtained by this process.

In practise, it has been found desirable to plate alternate layers of the gold-silver and indium and when all the layers have been plated, to diffuse for a suitable length of time, and at a suitable temperature whereby the metals of the layers intimately mix or alloy into a homogeneous single layer.

In carrying out the process in its entirety, the base metal, such as nickel silver, is first thoroughly cleaned. A thorough cleaning of the base involves successive application of a number of cleaning steps which are well known. An advantageous cleaning is obtained by subjecting the base metal to the following:—

- (1) Hot boiling soap solution. 86
- (2) Hot water rinse.
- (3) Hot mineral cleaner.
- (4) Cold running water rinse.
- (5) Alkali electric cleaner.
- (6) Cold running water rinse. 85
- (7) Dilute hydrochloric acid dip.
- (8) Cold running water rinse.

After this treatment, a very thin plate of nickel may be applied in any suitable manner and the base again subjected to a cold running water rinse.

The base is now advantageously subjected to a silver strike for about 8 seconds in a solution containing about ¼ ounces of silver per gallon in the form of potassium salts and 9 or 10 ounces of free potassium cyanide. This treatment produces a very thin silver layer on the base surface, giving a silver interior surface, and conditions said surface for the application of the heavier gold-silver and indium plates.

The gold-silver plating is now applied to about 25 millionths of an inch (0.000025) and the article then rinsed in cold water. It is then subjected to treatment in the indium bath to obtain an indium layer of about 20 millionths of an inch (0.000020). 105 At this point, a very thin layer of silver and indium may advantageously be applied and, in one practical method, the result is accomplished by a strike in a bath containing ¼ ounces of silver per gallon in the form of cyanide salts, about 1 110

ounce of indium per gallon in the form of cyanide salts, about  $\frac{1}{2}$  ounce of dextrose and about 10 ounces of free potassium cyanide per gallon. The current density is about  $\frac{1}{2}$  ampere per square inch for a short time.

The article is now subjected to another gold-silver plating to about 0.000025 inches and, following this, may be subjected to successive platings of indium and gold-silver with the intermediate silver-indium strikes and rinses until the desired thickness of plate has been built up. The application of successive steps for about ten (10) times has been found to give satisfactory results.

After the successive platings as above outlined, the produce is subjected to a diffusing process to cause the metals to alloy or mix intimately. The diffusion of the indium occurs at or about its melting point. The diffusing process is most advantageously carried out in two steps, the first step being a seasoning or readjustment to start the diffusion between the layers and the second step the complete diffusion of the layers together. In one practical species of the process, the first step is carried on with a preliminary heating at 110° C. for about 8 hours. The second is performed in an oven at 165° C. for about 18 hours. In this way, a very satisfactory homogeneous plate is produced.

With the compositions and thicknesses discussed, the final coating contains about 36% indium, 8½% gold and 55½% silver. These ratios may be varied as desired by changes in the original compositions and thicknesses.

This surface alloy is non-tarnishing and has a color simulating pure silver. It may be applied to base metals of various kinds and may be applied to silver itself, for example, to impart preservative surface coatings to precious silver articles.

In lieu of plating the silver and gold simultaneously and the indium separately, the silver and indium may be plated simultaneously, for example, by a bath such as described or otherwise, and the gold plated separately, the layers being built up alternately and the metals then intimately mixed or alloyed by diffusion.

Metals other than gold might be employed to modify the objectionable indium color and to give a more pleasing color where real silver color is not necessarily desired.

By way of example, an alloy may be of silver, palladium and indium and produced by plating the silver and palladium simultaneously and the indium separately in alternate superposed layers and then diffusing.

A suitable palladium-silver plating bath is as follows:—

Ounces per gallon

|                          |     |
|--------------------------|-----|
| Palladium (in cyanide)   | 0.8 |
| Potassium cyanide (free) | 5.0 |
| Potassium carbonate      | 5.0 |
| Potassium nitrate        | 1.0 |
| Silver                   | 1.0 |

The plating occurs with very little agitation at a current density of about 0.1 ampere per square inch. It is likely that, by having a much larger proportion of palladium, better deposits may be secured by means of agitation.

An intimate mixture or alloy may also be of silver, cadmium and indium and produced, for example, by plating the silver and cadmium simul-

taneously and the indium separately in alternate layers and then diffusing.

A suitable cadmium-silver plating bath is as follows:—

|                   | Ounces per gallon | 80 |
|-------------------|-------------------|----|
| Cadmium           | 0.8               |    |
| Silver            | 2.4               |    |
| Potassium cyanide | 2.4               |    |

This bath with a current density of 0.3 amperes per square inch gave 54% silver and 46% cadmium in the deposit and with a current density of 0.5 amperes per square inch 27% silver and 73% cadmium. Practically any mixture of the metals can be plated from a cyanide bath.

Another intimate mixture or alloy may be of silver, copper and indium and may be produced by plating the silver and copper simultaneously and the indium separately in alternate layers and then diffusing.

To obtain a suitable copper-silver bath, 250 grams of copper cyanide are mixed with 300 grams of potassium cyanide and 500 cubic centimeters of water added and the mixture stirred until the maximum amount of copper cyanide is dissolved. The solution is filtered and made up to two liters. The solution is a clear, light amber colored liquid, from which, when cold, a small quantity of white crystalline material is precipitated. This precipitate is the double cyanide of copper and potassium and dissolves when the solution is warmed. To this solution, silver is added in the form of silver potassium cyanide with a slight excess of potassium cyanide. The added solution is prepared by mixing 50 grams of silver cyanide and 50 grams of potassium cyanide and adding enough water to give 375 cubic centimeters solution. The above ingredients can probably be varied within wide limits, but the example given has been found to give good deposits.

It will be noted that silver, gold and copper are in the same group and sub-group of the periodic system, viz: group 1 sub-group, or family, B, so that gold and copper may be designated generically as metals other than silver of the same group and sub-group as silver.

What is claimed is:

1. A non-tarnishing intimate mixture or alloy having a color simulating silver comprising indium, gold and silver substantially in the ratio of about 36% indium, 8½% gold and 55½% silver.

2. A non-tarnishing mixture or alloy consisting of silver, indium and a color-modifying metal selected from the group consisting of gold, palladium, cadmium, and copper, the silver constituting more than 50% by weight of the total alloy, the indium and the color-modifying metal constituting substantially the entire remainder, the amount of indium present being in excess of the amount of color-modifying metal present.

3. A non-tarnishing intimate mixture or alloy consisting principally of silver, indium and a color-modifying metal selected from the group consisting of gold, palladium, cadmium and copper, the silver constituting more than 50% of the total alloy, the indium about 36% and the color-modifying metal constituting substantially the entire remainder.

WILLIAM S. MURRAY.  
DANIEL GRAY.